

# UNITED STATES PATENT OFFICE.

JAMES CLAUSEN, OF NEW YORK, N. Y.

## IMPROVEMENT IN LIQUID COMPOUNDS FOR BURNISHING LEATHER GOODS.

Specification forming part of Letters Patent No. **155,860**, dated October 13, 1874; application filed September 12, 1874.

*To all whom it may concern:*

Be it known that I, JAMES CLAUSEN, of New York city, in the county and State of New York, have invented a new and Improved Liquid Compound for Burnishing Leather Goods, of which the following is a specification:

The object of my invention is to furnish, for the purpose of burnishing and finishing the shanks, heels, sole edges of boots, shoes, and other leather articles, a compound which, if added in small quantities to the common burnishing-ink, imparts a deeper color to the same, and preserves a clear black luster for any length of time thereon.

The main defect of the ink generally used for blacking the shanks and other parts of the boots and shoes is that the same soon loses its original shining black color and takes a grayish hue, especially when the goods are kept stored for some time, presenting thereby a less attractive appearance.

My invention consists of an extract of nutgalls and logwood boiled with castile soap and a small quantity of glycerine, which is mixed with the ink, rendering the same very durable, and appearing with a deep and bright black color for any length of time.

The ingredients and the proportions in which the compound is prepared are as follows: Eight parts of ground nutgalls and ten parts of extract of logwood are boiled up in a suitable quantity of water, under the addition of four parts of castile soap and a small quantity of glycerine, until a liquid of easily-flowing consistency is produced. A few drops of this liquid are mixed with the common ink used for burnishing and finishing leather goods, the ink becoming thereby of superior blacking quality, and imparting a permanent and substantial shine to the parts prepared therewith.

Having thus described my invention, what I claim as new, and desire to secure by Letters Patent, is—

The liquid compound to be used for burnishing and finishing boots, shoes, and other leather goods, produced of ground nutgalls, extract of logwood, castile soap, and glycerine, mixed in boiling water, for being added to the common burnishing-ink in use, substantially as and for the purpose set forth.

JAMES CLAUSEN.

Witnesses:

PAUL GOEPEL,  
T. B. MOSHER.